

April 25, 1933.

R. H. MCKEE

1,905,731

PROCESS OF DIGESTING PULP AND APPARATUS THEREFOR

Filed May 4, 1929

2 Sheets-Sheet 1



INVENTOR  
RALPH H. MCKEE  
O. Dr. Deller  
ATTORNEY

April 25, 1933.

R. H. McKEE

1,905,731

PROCESS OF DIGESTING PULP AND APPARATUS THEREFOR

Filed May 4, 1929

2 Sheets-Sheet. 2



BY

INVENTOR  
RALPH H. McKEE  
O. J. Deller  
ATTORNEY

## UNITED STATES PATENT OFFICE

RALPH H. MCKEE, OF JERSEY CITY, NEW JERSEY

## PROCESS OF DIGESTING PULP AND APPARATUS THEREFOR

Application filed May 4, 1929. Serial No. 360,341.

The present invention relates to the art of digesting pulp, and more particularly to an improved process of digesting pulp and an apparatus therefor.

It has been the customary practice heretofore to cook wood chips in a digester provided with a central, single steam inlet which was located adjacent to the discharge outlet at the bottom of the digester. With this arrangement, the injected steam with heated cooking liquor passed up through the central portion of the digester to the top thereof, then outwardly toward the periphery of the digester, and finally downwardly to the bottom of the digester. This circulation of cooking liquor continued as long as steam was injected into the mass of wood chips and cooking liquor. The temperature, as is well known, was highest in the center of the digester and was lowest in the region adjacent the periphery thereof. As the cooking liquor descended in the peripheral regions of the digester, the liquor was cooled still more due to radiation and conduction heat losses. This tended to accentuate the temperature differences within the mass of digesting pulp and to effect a detrimental non-uniformity in operating conditions. Due to the non-uniformity of thermal conditions there was a tendency for the digester to become overheated to such an extent that the acid of the cooking liquor was decomposed and that a portion of the wood chips became brown and remained raw. When superheated steam was used, the non-uniformity and overheating within the digester were accentuated and the yield of good pulp was lower and the amount of screenings, due to brown and raw chips, was higher. Many attempts have been made to remedy the aforesaid disadvantages, particularly local overheating and decomposition of the acid of the cooking liquor with their consequent detrimental results, but none have, as far as I am aware, satisfactorily and successfully provided a commercially practical and efficient process and apparatus. The suggestions thus far made concerned themselves with attempts to modify the standard method and to adhere substantially to the centrally heated circula-

tion of liquor in either an upward or a downward direction and with either internal or external heating rather than any radical or fundamental departure from the standard digesting process.

In accordance with my discovery, however, I contemplate a basic departure from the standard pulp digesting method and the provision of a process which overcomes fundamental defects inherent in the standard method. It is also within the contemplation of my discovery to provide a process of digesting pulp which gives a practically even distribution of heat throughout the digesters and a uniformity of chemical action of cooking liquor on the mass of wood chips and which has practically no danger of local overheating and avoids dead cold spaces with resultant uncooked chips. A further object of my invention is to provide a pulp digesting process which permits keeping more sulfur dioxide in solution in the cooking liquor due to the maintenance of an average low temperature and which effects a thorough penetration of wood chips before the critical temperature of about 120° C. is reached. Another object of my invention is to provide a process which prevents the tendency toward the formation of excessive temperatures that drive off too much SO<sub>2</sub> with a concomitant dilution of the acid in the cooking liquor toward the terminal period of the digestion of chips, which process has very little tendency to liberate gases and to cause shocks and noises in the digester and which is simple, economical and practical.

Other features and objects of my invention will become apparent from the following description taken in conjunction with the accompanying drawings, in which:

Fig. 1 is an elevational view, partly in section, of my improved digester used for carrying my new process into practice;

Fig. 2 is a sectional view taken on the line 2-2 of Fig. 1;

Fig. 3 is a view similar to Fig. 1 of a modified digester employing electrical heat;

Fig. 4 illustrates diagrammatically a di-

55

60

65

70

75

80

85

90

95

100

gester provided with my new circulation system; and

Figs. 5 and 6 are diagrammatic views illustrating the circulating systems heretofore used in prior digesters.

Referring more particularly to Fig. 1, the numeral 1 designates the shell of my improved pulp digester. The shell preferably consists of a main cylindrical intermediate portion 2 and a conical bottom and top 3, 3. Any suitable construction may be employed for the shell but I prefer to construct it of riveted or welded plates of a material resistant to the action of sulfite cooking liquor. A material of this type, for example, is described in my Patent No. 1,841,752, relating to Industrial chemical vessels issued on January 19, 1932. This material consists of an alloy of iron containing about 15% to 20% chromium and about 7.5% to 10% nickel. For instance, an alloy steel containing about 18% chromium, about 8% nickel, say under 0.20% carbon, about 0.05% manganese and 0.50% silicon, and the remainder iron is a suitable material.

The conical top 3 is preferably provided with a neck 4 which is flared into a flat annular mouth 5. Seated upon mouth 5 is a cover 6 which is bolted thereto by means of a plurality of swing bolts 7. These bolts may be of a suitable type, as is well known in the art. In my improved digester I prefer to employ a solid cover which does not have the customary outlet pipes and the like incorporated therein, which can be easily made from the material referred to hereinabove and which can be conveniently handled in daily operations and use.

In neck 4 or conical top 3 a well-known top relief line 8 containing valve 8' is provided in an appropriate manner. The inlet port 9 within the digester is protected by a strainer 10 having perforations, say about  $\frac{1}{8}$ " in size. A second relief line 11, commonly known as the side relief, contains a suitable valve 12 and projects from the upper part of the main cylindrical portion 2 as may be seen from Fig. 1. A strainer 13 having a construction similar to strainer 10 is secured over inlet 14 of the side relief line. The purpose and function of these valves are well known to those skilled in the art and, consequently, no detailed description is necessary.

The shell 1 is preferably supported by a plurality of legs or standards 15 herein shown as six in number. Other suitable supporting means, however, may be employed for mounting the digester shell as one skilled in the art will readily understand. Mounted around the upper portion of the conical bottom 3 and preferably above the standards 15 is a steam feed pipe 16 which supplies a plurality of steam jets 17 within the digester shell with steam. These

steam jets are preferably located adjacent to the periphery of the bottom of the main cylinder 2 and are pointed upwardly. Any appropriate number of steam jets may be used but I prefer to employ three or more and I have illustrated a digester with six steam jets. A valve 18 may be provided for each steam jet and/or a main valve 19 may be incorporated in the main steam line 20.

The base of the conical bottom 3 terminates in an outlet port 21 to which is secured an outlet fitting 22, such as a right angle pipe section, by a plurality of bolts, for instance, or other suitable means. Associated with the outlet fitting is a customary blow-off valve 23 for controlling the discharge of the contents from the digester to outlet line 24 which is directed at a well known target (not shown) as is usual in the sulfite pulp art. When the digester is made of my alloy steel referred to hereinabove or of a metal having similar properties, I prefer to make the conical bottom 3 shallow in contradistinction to the steep bottoms of conventional digesters. The angle of the conical bottom from the horizontal may vary depending upon the particular circumstances but an angle of, say,  $30^\circ$  is satisfactory. Ordinarily the angle of conventional digesters is about  $70^\circ$ . With my improved digester there will be a saving of material and of labor and due to its smooth inner surface there will be less loss in blowing (i. e. in emptying the digester) due to the bridging or adherence of solid material to the surface of the digester.

My improved pulp digester is provided with the customary and conventional auxiliaries. For instance, a sampling cock 25 to draw off samples of cooking liquor for analysis is shown mounted at an intermediate point on the side of the main cylinder 2. Positioned above the sampling cock 25 is the usual thermometer well 26 which is intended for the reception of a thermometer for measuring the temperatures of cooking liquor within the digester. In view of the fact that other auxiliaries are well known, it is not necessary to illustrate them. For instance, external insulation may be used, as it is in some cases, to lag the outside of the digester so as to prevent the loss of excessive quantities of heat.

A modification of my improved digester is illustrated in Fig. 3. The entire construction of the modified digester is the same as that described hereinabove with the exception that electrical means are employed to furnish the heat for the modified digester instead of steam jets. It will not be necessary to repeat the description of the digester depicted in Figs. 1 and 2.

The electrical heating arrangement provided for digester 1 may be of an appropriate type. For instance, an electrical resistor

heating device may be applied to the digester or an electrical induction heating device may be used. Either of these types, as those skilled in the art will readily understand, can be applied to a digester with all of the necessary auxiliaries. I prefer to employ the electrical induction heating for a variety of reasons and I have illustrated this type in Fig. 3.

10. An annular metal shelf 30 supported by a plurality of strong brackets 31 is affixed, preferably by welding, to the lower portion of the main cylindrical shell 2 adjacent to conical bottom 3. Upon this shelf a wall 32 of electrical insulating material is built up to a suitable height, say four feet or so. Any suitable electrical insulating material may be employed but I prefer to use carborundum (silicon carbide) bricks. The 15 wall 32 is preferably built up of alternate rows 33 and 34 which are made of bricks laid on their flat side and bricks laid on their edge as one will readily understand. By laying the bricks in this manner channels 36 are formed between adjacent rows 33. In order to provide a connection between adjacent channels 36 one or more bricks are broken or cut off as indicated by openings 35, so that they do not project beyond the face of the bricks in rows 34. An 20 electrical conductor 37 can be wound in channels 36 so as to extend from the bottom of wall 32 to the top thereof. The ends 38 and 39 of conductor 37 can be secured in binding posts 40 and 41 respectively. These 25 binding posts act as terminals of the electrical conductor to which a source of alternating electric current can be connected. Of course, the source of current is provided 30 with well-known auxiliaries for the supply of proper and controlled electrical energy.

The total number of turns of conductor 37 on wall 32 and the number of turns in each channel will vary with the particular circumstances as those skilled in the art of electric induction furnaces will readily understand. For instance, the number of turns will vary according to the voltage of the source of alternating current feeding the 45 conductor 37 (i. e. to the electrical current which the voltage forces through the conductor), to the heat required by the cooking liquor and the mass of wood chips within the digester, to the size of the digester, to the rate and temperatures at which the heating is to be conducted and to other related factors. Then again in the preferred embodiment conductor 37 is made as a hollow pipe through which cooling water may be 50 passed.

When alternating electric current is supplied to conductor 36 induced currents are set up in the steel shell of the digester. These induced currents, as is well known, 55 cause the evolution of heat. In view of the

fact that this heat is effective within the walls of the digester shell it is transmitted to cooking liquor contained in the digester via a large peripheral area. As cooking liquor becomes heated, due to its contact 70 with the inner heated surface of the digester, it rises upwardly to the upper portion of the body of cooking liquor where it then moves toward the central area thereof. Upon reaching the central area it moves 75 downwardly and takes the path as indicated by the arrows within the digester in Fig. 3. This circulation continues as long as heat is applied to the electrical heating system and functions in the same manner as in my 80 steamheated digester, all as will be more fully described hereinafter.

When electrical resistance heating is to be employed, conductor 37 may be made, for instance, of the well known resistance alloy 85 known as nichrome and described in U. S. Patent Number 811,859 to Albert W. Marsh. With the passage of electrical current through nichrome conductor 37, heat is generated within the conductor and is given off 90 to the surrounding environment. Since bricks made of silicon carbide are good thermal conductors, the heat generated in the nichrome conductor is readily transmitted to the shell of the digester and the 95 contents thereof. In this manner the cooking liquor within the digester can be conveniently brought to the desired temperatures within the predetermined period of time as set forth hereinafter. Of course, 100 the outside of wall 32 may be lagged with an insulating brick made of infusorial earth or the like so as to conserve heat and prevent its loss by dissipation to the atmosphere.

In carrying my improved process of digesting pulp into practice I prefer to use the apparatus described hereinabove although any suitable pulp digester may be employed. A typical run embodying my process may 110 be described in connection with my digester illustrated in Figs. 1 and 2 as follows: The digester is first filled with wood chips and a cooking acid or liquor carrying about 4% of free sulfur dioxide and 1% of combined 115 sulfur dioxide (calculated as  $\text{CaSO}_3$ ) is run into the digester until the chips are about covered by the cooking liquor. The digester is closed with its cover 6 and proper valve connections are made via valves 18 and 19 120 to permit a flow of steam from the main steam line 20 to the peripheral steam jets 17 and into the cooking liquor contained in the digester. Steam is preferably turned on at such a rate that the digester will reach a 125 temperature of  $115^\circ \text{ C.}$  in about two hours. After a temperature of  $115^\circ \text{ C.}$  has been reached, steam is then slowly injected via the peripheral jets until a temperature of about  $145^\circ \text{ C.}$  is reached. This will take 130

about six additional hours and will be accompanied by "relieving" the digester in the well known manner from time to time by means of the "top relief" line 8. Sometimes it will be desirable and necessary to use the "side relief" line 11 from the digester in case the temperature rises too rapidly. When the temperature has reached 145° C. the steam is almost turned off and the cooking continued at this temperature for about one and a half hours longer. This is accompanied by relief of the "dry gas", as is customary in pulp digestion. During the last hour the pressure will gradually decrease and at the end of the period when the pressure gauge shows a pressure of only about twenty to thirty pounds above atmospheric pressure, the bottom valve 23 is opened and the contents of the digester blown into the blowpit.

The circulation of cooking liquor within a pulp digester when proceeding in accordance with my process may be clearly observed from Fig. 4 wherein a pulp digester is diagrammatically illustrated. Steam entering the digester via the peripheral steam jets causes a substantially vertical upward flow of cooking liquor contiguous to the inner periphery of the digester shall to the upper portion of the body of cooking liquor. During this upward flow the liquor is being heated by the steam coming from the steam jets so that the peripheral portion of the cooking mass is slightly hotter than the central portion. At the upper portion of the digester the cooking liquor flows toward the center of the digester and then downwardly through the central portion of the digester to the bottom cone thereof. The cooking liquor thereafter flows upwardly along the walls of the digester as indicated by the arrows in Fig. 4. With circulation of the aforesaid type it is possible to maintain temperature conditions substantially uniform throughout the body of the cooking liquor.

In utilizing my process thermal conditions are maintained substantially uniform through the digester and the contents thereof can be heated to, say, about 100° C. without any portion becoming overheated locally to, say, about 120° C. or without any spots or portions remaining cold. By effecting a uniform heating a thorough penetration of the wood chips by the cooking liquor can be obtained. After the penetration of the chips with cooking liquor, which occurs in my process at about 100° C. within about the first two hours, the entire contents of the digester can be heated to a cooking temperature of about 145° C. By maintaining the cooking temperature for a suitable period of, say, about six hours, the entire charge is thoroughly cooked without having burnt pulp, i. e. darkened and undigested

In this manner I am able to obtain a maximum yield of good pulp and a minimum amount of burnt pulp.

In the digesting of pulp it is now believed that weak acid salt, such a calcium bisulfite, when the temperature is high (say about 120° C. or above), is largely hydrolyzed to give free lime ( $Ca(OH)_2$ ) and sulfur dioxide ( $SO_2$ ) which is in solution and not sulfurous acid ( $H_2SO_3$ ). When this occurs before penetration of the wood chips, the cooking acid is decomposed and the chips are burnt and come out of the digester brown in color and are discarded when the pulp is screened. These disadvantages are avoided by the use of my process. It is my belief that in digesting wood chips in accordance with my invention the calcium bisulfite solution containing sulfurous acid has ample opportunity to wet and to diffuse into the fibers of the wood chips before the temperature for chemical action is reached. Under usual conditions this temperature is about 120° C.

The circulation of the conventional method of digesting pulp heretofore employed is illustrated diagrammatically in Fig. 5. Steam was usually injected via a single central jet located in the bottom cone or via several jets located within the central region so that a vertically upward flow of cooking liquor was effected at the center of the digester. Upon reaching the top of the cooking liquor, the flow would be directed towards the periphery of the digester and would then pass downwardly adjacent to the walls of the digester to the bottom of the cone where the rising steam would carry the cooking liquor upwardly again as may be clearly seen from the arrows in Fig. 5. With this type of circulation the center of the digester was hottest and the outside was coldest. Due to the large surface on the outside of the digester, the heat loss was increased and the difference in temperature between the peripheral portions of the body of cooking liquor and the central portion was accentuated. For example, differences of temperature of about 50° C. have been observed even in the second hour of heating. During later periods of a run differences of temperature of about 15 to 20° C. were quite common. Ordinarily the center of the digester was 10° C. or more hotter than portions of the periphery, even when handled by the most experienced operators. With non-uniformity of thermal conditions within the digester, some portions thereof were overheated and in some cases a temperature of 120° C. was reached before a thorough penetration of the wood chips occurred. Due to the local overheating before the whole digester reached a condition where the wood chips were thoroughly penetrated by cooking liquor, burnt pulp was produced, i. e. pulp containing darkened and undigested

wood chips. The central injection of steam also has the disadvantage of causing clashing of the liquor surfaces against each other as a result of the condensation of the injected steam. Attempts have been made to overcome the non-uniformity of thermal conditions in pulp digesters but, as far as I am aware, none have been satisfactory or successful. A typical example of one of the

10 proposed modified methods is diagrammatically illustrated in Fig. 6. Instead of injecting steam directly into the digester to cause the circulation a centrifugal pump C was used to cause a forced circulation of the 15 cooking liquor through the digester as depicted by the arrows in Fig. 6. In some cases the cooking liquor was heated in an external heater H instead of by direct injection of steam into the body of the cooking 20 liquor. In either case there was a tendency for the central portions to be hotter than the peripheral portions of the digester and a non-uniformity of thermal conditions was present within the digester.

25 With my improved method of digesting pulp involving heating by a plurality of peripherally-located steam jets, the contents of the digester are far more evenly heated and the thermal conditions within 30 the digester are practically uniform. The differences of temperature with my system of heating and circulating will be much less than in prior methods noted hereinabove and will be, for instance, of the order of, say 35  $\frac{1}{4}$  of those mentioned heretofore. My use of steam injection at a plurality of peripherally-located points not only obviates the danger of local overheating but also avoids having dead cold spaces with resultant uncooked chips. More sulfur dioxide can be 40 kept in solution with my method due to the uniformity of temperature and the maintenance of an average low temperature.

45 It is to be observed that by the use of my digester provided with an electrical heater, it is possible to obtain in a convenient manner a good control over the heating of the cooking liquor and to effect a peripherally upward and a centrally downward circulation 50 of the cooking liquor. As no steam is introduced into the body of cooking liquor with electrical heat, there is no tendency to dilute the cooking liquor during the run with a consequent weakening of the acid 55 in the liquor. The strength of the cooking liquor is consequently protected against detrimental dilution throughout the run.

60 While I have described the process as exclusively for making sulfite pulp it is to be observed that my method is equally applicable to pulp made by the soda process or by the kraft process (sulfate process).

65 Although certain specific embodiments of my digester have been described, it is to be understood that the invention is not re-

stricted to such particular embodiments. For instance, the electrical heating may be replaced by a jacket for heating by oil or other heated fluid. Various other modifications in detail and in the arrangement may 70 be made by those skilled in the art without departing from the invention as defined in the claims.

What I claim is:

1. A pulp digester having electrical heat- 75 ing means.

2. A pulp digester having a main body portion and a top and bottom, and electrical heating means mounted around the lower portion of said main body portion and adapted to heat cooking liquor within said digester at the outermost peripheral portions of said digester whereby an upward flow of cooking liquor adjacent to said outermost peripheral portions is effected. 80

3. A pulp digester having a metallic shell free from an inner lining and constituted of an alloy steel containing about 7.5 to 10% nickel and about 15% to 20% chromium and of a main body portion and a top and bottom, and having an electrical heating means mounted around the lower portion of said shell whereby heat is transmitted through said metallic shell directly to cooking 85 liquor. 90

4. A pulp digester comprising a main cylindrical body, a top provided with a charging mouth and cover and a relief valve; a shallow conical bottom devoid of a strainer; a free, unobstructed outlet located in the central region of said bottom and capable of permitting the discharge of cooked pulp by blowing; a plurality of steam jets mounted adjacent to the inner surface of said cylindrical body in direct contact with chips and cooking liquor in the digester and not lower than a region adjacent to the junction of the cylindrical body and the conical bottom; said steam jets extending upwardly in approximately a vertical direction and being capable of effecting a maximum speed of flow of cooking liquor contiguous to the inner surface of said cylindrical body; and valve means to control steam flowing to said jets. 100 105 110

5. A pulp digester comprising a main cylindrical body composed of an alloy, nickel-chromium steel and having the inner surface thereof free from lining material, a top made of said alloy steel and provided with a charging mouth and cover and a relief valve; a shallow conical bottom devoid of a strainer and made of said alloy steel, said conical bottom having an angle of approximately 30°; a free, unobstructed outlet located in the central region of said bottom and capable of permitting the discharge of cooked pulp by blowing; a plurality of steam jets mounted adjacent to the inner surface of said cylindrical body in direct contact 115 120 125 130

- with chips and cooking liquor in the digester and not lower than a region adjacent to the junction of the cylindrical body and the conical bottom; said steam jets extending 5 upward in approximately a vertical direction and being capable of effecting a maximum speed of flow of cooking liquor contiguous to the inner surface of said cylindrical body; and valve means to control 10 steam flowing to said jets.
6. A pulp digester comprising a main cylindrical body, a top provided with a charging mouth and cover and a relief valve; a shallow conical bottom devoid of a strainer; 15 a free, unobstructed outlet located in the central region of said bottom and capable of permitting the discharge of cooked pulp by blowing; heated means provided adjacent to the cylindrical body and located not lower 20 than the region adjacent to the junction of the cylindrical body and the conical bottom, said heating means being in direct contact with chips and cooking liquor in the digestor and being arranged to heat cooking liquor 25 in a region adjacent to the inner surface to a temperature higher than any other region within the digestor and to give to said cooking liquor in the region contiguous to the inner periphery of said cylindrical body a 30 speed of flow in an upward vertical direction higher than any other region within said digester whereby an upward flow of cooking liquor only takes place adjacent to the inner periphery of the cylindrical body 35 and a downward flow only occurs in the central portion of the digester; and means to control said heating means. 40
7. The process of digesting pulp in a digester having a cylindrical body and a conical top and bottom which comprises charging an unobstructed space in a digester with wood chips and cooking liquor, heating a region closely adjacent to the inner periphery of the cylindrical body to give to said 45 cooking liquor in said region a higher temperature and a greater speed of upward, vertical flow than any other region within said digester, limiting the upward flow of cooking liquor in a region adjacent to the inner periphery of said cylindrical body and a downward flow occurs in the central portion of said digester, maintaining the cooking liquor and the wood chips adjacent to the inner periphery of said body hotter than 50 the chips and liquor in the central portion, continuing the heating until the pulp is digested and then discharging the cooked pulp by blowing. 55
8. The process of digesting pulp in a digester having a cylindrical body and a conical top and bottom which comprises charging an unobstructed space in a digester with wood chips and cooking liquor, heating a region closely adjacent to the inner periphery of the cylindrical body to give to said 60
- cooking liquor in said region a higher temperature and a greater speed of upward, vertical flow than any other region within said digester, effecting said heating by injecting steam in direct contact with chips and liquor closely adjacent to the inner periphery of the digester, limited the upward flow of cooking liquor in a region adjacent to the inner periphery of said cylindrical body so that a downward flow occurs in the central portion of said digester, maintaining the cooking liquor and the wood chips adjacent to the inner periphery of said body hotter than the chips and liquor in the central portion, continuing the heating until the pulp is digested and then discharging the cooked pulp by blowing. 70
- In testimony whereof I have hereunto set my hand.
- RALPH H. McKEE. 85
- 90
- 95
- 100
- 105
- 110
- 115
- 120
- 125
- 130

**CERTIFICATE OF CORRECTION.**

**Patent No. 1,905,731.**

**April 25, 1933.**

**RALPH H. McKEE.**

It is hereby certified that error appears in the printed specification of the above numbered patent requiring correction as follows: Page 2, line 130, for "resister" read resistor; page 4, line 29, for "shall" read shell; line 70, after "that" insert the article "a" and in the same line for "a" read as; page 6, line 18, claim 6, for "heated" read heating; and line 72, claim 8, for "limited" read limiting; and that the said Letters Patent should be read with these corrections therein that the same may conform to the record of the case in the Patent Office.

Signed and sealed this 21st day of November, A. D. 1933.

**F. M. Hopkins**

**(Seal)**

**Acting Commissioner of Patents.**